

## UNITED STATES PATENT OFFICE

2,017,646

BATH FOR THE ELECTRODEPOSITING  
OF COBALT

Henri Berger, Paris, France

No Drawing. Application June 7, 1934, Serial  
No. 729,418. In France October 3, 1933

4 Claims. (Cl. 204—1)

## Example

Various solutions have been proposed up to the present time for electroplating metals and cobalt, either with a view to hardening the surface of the metal (cobalting of printing plates), or in order to obtain surfaces having a maximum reflecting power (cobalting of metallic mirrors and reflectors), or merely in order to decorate the metal that is treated by the electrodepositing process or to protect it against oxidation.

- 10 All the electrolytes that have been utilized up to this time consisted chiefly of ordinary cobalt sulfate or of ammoniacal cobalt sulfate, with or without the addition of earth or alkali-earth metals, these additions being intended to increase 15 the conductivity or the power of penetration or to promote anodic corrosion.

The drawbacks of such solutions are that they can be utilized only with limited current densities and, especially, that they only permit the use 20 of low tensions, under which conditions it is possible to obtain only blackish deposits, either granular or little adhesive, which most often necessitate a preliminary coppering or brassing when the electrodepositing is to be effected on iron or 25 steel.

It has already been suggested to utilize as electrolyte a solution containing chiefly cobalt chloride. But up to now such solutions have yielded 30 only defective cobalt deposits, even with the addition of earth or alkali-earth metal salts, generally employed for improving them. The percentage of metal in such baths rapidly decreases due to anodic polarization and there results an irregular working, which makes it necessary to 35 frequently add cobalt chloride.

The object of the present invention is to provide an electrolytic bath which does away with these drawbacks.

To this effect, the electrolyte that is utilized consists chiefly of cobalt chloride  $\text{CoCl}_2 \cdot 6\text{H}_2\text{O}$ , but according to the present invention, there is added to the solution an alkaline bifluoride with, eventually, boric acid. The latter is intended to serve 40 to maintain a normal acidity of the bath.

In such baths, the anodic corrosion is perfectly regular, which maintains the metallic percentage at its normal value, so that the operation is very regular and very easy to control.

An aqueous solution containing from 50 to 600 grammes of cobalt chloride per litre and from 10 to 120 grammes of ammonium bifluoride makes it possible to obtain very white cobalt deposits, which are perfectly adhesive, even when made directly on iron and steel and which can be brightly polished, the conditions of the operation being very much facilitated from the point of view of the current regulation.

As a matter of fact, experiments proved that, with a tension which may vary between  $2\frac{1}{2}$  and 6 volts and a density of current ranging between 2 and 15 amperes per square decimetre, with a normal interval between the electrodes, the deposit has a fine grain and is evenly white, very smooth and very supple. By raising the temperature of the bath, these figures are substantially increased, as in the case of nickel-plating.

The addition of boric acid to the bath above mentioned gives still better results. I may also, according to the invention, add to the electrolyte in question various products intended to give brightness to the deposit (colloids), or to avoid pitting (nitrates), in the usual proportions, these products being well known in the art of electrodepositing.

While I have described what I deem to be a practical example of the present invention, it should be well understood that I do not wish to be limited thereto as there might be changes made therein without departing from the principle of my invention as comprehended within the scope of the appended claims.

What I claim is:

1. A bath for the electro-depositing of cobalt containing cobalt chloride mixed with an alkaline bifluoride.

2. A bath for the electro-depositing of cobalt containing cobalt chloride mixed with an alkaline bifluoride and boric acid.

3. A bath for the electro-depositing of cobalt which contains from 50 to 600 grammes of cobalt chloride and from 10 to 200 grammes of an alkaline bifluoride per litre of water.

4. A bath according to claim 3 in which the alkaline bifluoride is ammonium bifluoride.

HENRI BERGER.